

Jan. 20, 1959

A. L. BREEN

2,869,967

BULKY YARN

Filed Aug. 23, 1957

4 Sheets-Sheet 1



*Fig. 2*



*Fig. 3*



*Fig. 4*



*Fig. 5*



*Fig. 8*



*Fig. 6*



*Fig. 9*



*Fig. 7*



INVENTOR

ALVIN L. BREEN

BY *Frank C. Hilberg*

ATTORNEY

Jan. 20, 1959

A. L. BREEN

2,869,967

BULKY YARN

Filed Aug. 23, 1957

4 Sheets-Sheet 2

*Fig. 10*



*Fig. 11*



*Fig. 19*



BY *Frank C. Helberg*

ATTORNEY

Jan. 20, 1959

A. L. BREEN

2,869,967

BULKY YARN

Filed Aug. 23, 1957

4 Sheets-Sheet 3

*Fig. 12*



*Fig. 13*



ALVIN L. BREEN

BY

*Frank C. Hulberg*

ATTORNEY

Jan. 20, 1959

A. L. BREEN

2,869,967

BULKY YARN

Filed Aug. 23, 1957

4 Sheets-Sheet 4

*Fig. 14*



*Fig. 15*



*Fig. 16*



*Fig. 17*



*Fig. 18*



INVENTOR  
ALVIN L. BREEN

BY

*Frank C. Tidberg*

ATTORNEY

# United States Patent Office

2,869,967

Patented Jan. 20, 1959

1

2,869,967

## BULKY YARN

Alvin L. Breen, West Chester, Pa., assignor to E. I. du Pont de Nemours and Company, Wilmington, Del., a corporation of Delaware

Application August 23, 1957, Serial No. 679,891

8 Claims. (Cl. 57—140)

This application is a continuation-in-part of my co-pending application, Serial No. 443,313, filed July 14, 1954, now abandoned.

This invention relates to treatment of yarn, or thread, to produce yarn of greatly increased bulk, and is more particularly concerned with the production of a bulky yarn composed of plurality of individually convoluted fibers and characterized by the presence of a multitude of ring-like loops and protruding fiber ends irregularly spaced along the yarn surface.

In my copending application, Serial No. 261,635, filed December 14, 1951, now Patent No. 2,783,609 I disclose the production of a novel bulky filament yarn having most of the desirable properties of ordinary spun staple yarn, but differing in being composed of substantially continuous filaments. In that yarn, bulk and an appearance resembling that of staple yarn is provided by a multitude of ring-like loops and other convolutions at random intervals along the filaments and irregularly spaced on different filaments. While this continuous filament structure is a distinct advantage for most purposes, there are textile uses which require a fuzzy, lofty or cashmere-like effect provided by a yarn which has a large number of protruding filament ends. A yarn having the combination of properties provided by free ends and bulk-giving filament convolutions would be desirable for such uses.

With the exception of silk, natural animal, vegetable and mineral fibers exist only in relatively short lengths. Yarn prepared from these natural fibers necessarily is composed of staple length fibers. Furthermore, large quantities of artificial continuous filaments are cut into staple before processing into yarn. Treatment of these staple yarns to introduce bulk-giving convolutions would be desirable regardless of whether or not free ends are required. When the desired effect requires protruding ends it would be highly desirable to provide a process for treating continuous filament yarn to impart both bulk and a multitude of protruding ends in one operation, thereby avoiding the expensive operations of cutting continuous filaments into staple and spinning the staple into yarn.

An object of this invention is to provide a yarn which has a large number of protruding free ends of fiber and has an enhanced bulk provided by filament convolutions of the type characterized by the presence of ring-like loops. Another object is to provide a spun staple yarn of improved bulk characterized by the presence of a multitude of ring-like loops and protruding fiber ends irregularly spaced along the yarn surface. A further object is to provide a process for preparing yarn of improved bulk from conventional spun staple yarn. An additional object is to provide a process for treating continuous filament yarn to provide greatly increased bulk and a covering of projecting fiber ends in one operation. Other objects of the invention will become apparent from the following description and claims.

In the drawings, which illustrate preferred embodiments of the invention,

2

Figure 1 is a side elevation of suitable apparatus for practicing the process of this invention,

Figure 2 is a side elevation, partially in section, of an alternative form of nozzle,

5 Figure 3 is an end view of the nozzle shown in Figure 2,

Figure 4 is a side elevation, partially in section, of another form of nozzle,

10 Figure 5 is a side view showing the appearance of untwisted treated yarn prepared from continuous filament yarn (enlarged about ten times),

Figure 6 is a similar enlarged view of untwisted treated yarn prepared from two plies of continuous filament yarn,

15 Figure 7 is a similar enlarged view of treated yarn prepared from a ply of continuous filament yarn and a ply of cotton yarn,

Figure 8 is a similar enlarged view of a treated yarn prepared from a single ply spun staple yarn,

19 Figure 9 is a similar enlarged view of a treated yarn prepared from a two ply spun staple yarn,

20 Figure 10 is a schematic view of the arrangement of the yarn feed, texturing jet, torque jet, take-up roll and wind-up,

Figure 11 is a schematic view of an alternate arrangement similar to Figure 10 but includes a draw roll with 25 a step roll and a draw pin,

Figure 12 is a self-explanatory alternate arrangement of Figure 10,

Figure 13 is a diagrammatic section of a flocking box 30 provided with a texturing jet,

Figure 14 is a schematic view of an arrangement of 35 yarn feed rolls, flocking box, pinch rolls and wind-up,

Figure 15 illustrates diagrammatically in isolated strands how the staple fibers are caught in loops introduced by a jet,

35 Figure 16 shows the staple secured in the loops of Figure 15 which have been drawn to lock the staple fiber in place,

Figure 17 shows the staple fiber flattened back against the load-bearing fiber in an isolated strand,

40 Figure 18 illustrates how some strands are wrapped around the filament bundle by the torque jet, and

Figure 19 represents a modification in which a T-shaped tube is used in place of the texturing jet. The T tube may be made of any smooth material such as glass, 45 stainless steel, or the like, and may vary in diameter from about  $\frac{1}{8}$ " to  $\frac{1}{2}$ ".

In accordance with this invention a novel yarn is provided which has a fuzzy to cashmere-like appearance resulting from a covering of projecting fiber ends and unusual bulk, as compared with staple yarns of the prior art, resulting from fibers which are convoluted into coils, loops and whorls at random intervals along their lengths and at irregular spacing on different fibers to provide a lateral interfiber spacing. The most obvious characteristics of the yarn are the combination of unusual bulkiness with the fuzzy covering provided by protruding fiber ends, but the yarn is also characterized by the presence of a multitude of ring-like loops and other convolutions in the fibers. The convolutions visible on the surface contribute desirable properties to the yarn, but the less obvious fiber convolutions within the yarn are even more important in producing bulk and resulting garment warmth of fabrics made from this yarn.

65 The characteristic loops in the yarn fibers have been described as "ring-like" because they are tiny complete loops formed by a fiber doubling back upon itself, crossing itself and then proceeding in substantially the original direction. In mathematics a curve of this type is said to have a crunode. Accordingly the characteristic loops will be more specifically defined as "crunodal loops," and loops of this type are intended unless otherwise indicated in the following specification and claims: The

majority of loops visible on the surface of the yarn are of a roughly circular shape and are properly described as ring-like. The crunodal loops inside of the yarn are not readily studied, but it is evident that pressure of surrounding filaments will tend to cause such loops to assume more complex shapes.

The fiber ends and convolutions maybe are held in place by a twist imparted to the yarn. A single ply yarn may have a **Z** or **S** twist. In a multiple ply yarn the individual plies are usually twisted in one direction and the plurality of plies are usually twisted together in the opposite direction, e. g., the plies may have a **Z** twist and the yarn may have an **S** twist. Unless the convolutions have been set, as by heating the convoluted yarn, the fibers will resume their original unconvoluted condition when the yarn is untwisted and taken apart; hence initially straight fibers will be recovered in a substantially straight condition. Of course, if the yarn fibers were initially crimped or wavy or curly, they would resume that condition on being separated from the yarn.

The yarn of this invention is prepared by a process which involves feeding yarn through a high velocity fluid jet, under conditions adapted to accomplish the double purpose of imparting bulk-giving convolutions and of providing a multitude of projecting filament ends, and then twisting the filaments together to hold the convolutions and filaments ends in place. In some respects the process resembles that of my copending application, Serial No. 261,635, now Patent No. 2,783,609. However, additional critical conditions must be observed to provide the desired covering of filament ends on the yarn surface.

The starting yarn may be composed of substantially continuous filaments or of staple length fibers, which may be natural fibers or artificial filaments cut to staple length, or the yarn may include two or more of these types.

When treating yarn composed of substantially continuous filaments in accordance with this invention, the yarn is fed through a jet operated under conditions such that the filaments are shattered at random intervals to provide the desired free ends of projecting fiber. In order to accomplish this, the jet must first open up the yarn. The filaments of an untwisted continuous filament yarn are readily separated by the turbulence created by a high velocity jet. Twisted yarn must be untwisted before the filaments can be separated, but this action can also be achieved by the jet. Under proper conditions the jet will apply sufficient false untwisting to the yarn filaments to permit the jet to open up the yarn, and this is true not only when the yarn is composed of a single twisted ply, but also when it is composed of a plurality of plies which are individually twisted. Once the yarn filaments are separated, suitable jet turbulence will whip the filaments about with such rapidity that the flex life of the material is quickly exceeded and some or many of the filaments are broken.

Operation of the jet at approximately sonic velocity, or near sonic velocity, will accomplish these objectives of opening up the yarn and whipping the filaments about sufficiently to shatter them into relatively short lengths. The distance the yarn travels through the jet should be less than the average length of the fibers produced by this shattering of continuous filaments, so that the fibers will not be removed from the yarn to an objectionable extent. After the yarn is withdrawn from the jet it is twisted to hold the resulting fibers and convolutions in place. The severity of the shattering effect will vary with the flex life of the filament material, under otherwise similar conditions, but the structure resulting from the treatment can be controlled by the rate at which the yarn is passed through the jet.

Preparation of the yarn of this invention from staple yarn is simpler in at least one respect, since filament-shattering is not required, but unexpected difficulties must be overcome or else the yarn is either torn to pieces or is substantially unaffected by the treatment.

The fibers of staple yarn must be held in place by a twist in the yarn, but the yarn must be untwisted while in the jet for the treatment to have appreciable effect. At near sonic velocities the jet has been found to apply a substantial untwisting torque as well as considerable tension to the yarn. If the yarn is permitted to untwist in response to this torque for a distance which exceeds the fiber length, the draft yield strength of the yarn is reduced to such an extent that the accompanying jet tension is sufficient to pull the yarn apart. When the yarn is fed through the jet to a windup, it has been found that the untwisting action of the jet is limited to the length of yarn between the feed and windup devices. In other words, the jet torque applies a false untwist to the yarn. The extent of this false untwisting action is inversely proportional to the tension applied to the yarn between feed and windup, since tension imposes a torque which opposes the jet torque. Hence the false untwist can be controlled by increasing the tension, but this does not solve the difficulty because the total of the jet tension and windup tension then exceeds the yarn strength.

In accordance with this invention it has been found that yarn which consists wholly or in part of staple-length fibers held in place by a yarn twist can be processed efficiently when feeding the yarn to a high velocity fluid jet operated to apply a false untwist to the yarn, by snubbing the yarn passing to the jet to prevent the untwist from backing up, and again snubbing the yarn leaving the jet to prevent the untwist from carrying forward, the distance between the two snubbing points being less than the length of the staple fibers and preferably being arranged to restrict the false untwist to an effective distance of less than one-half the length of the staple fibers. The required snubbing may be accomplished by dragging the yarn over fixed surfaces, which may be the yarn entrance and exit surfaces of the jet nozzle. The yarn leaving the jet can be snubbed by directing it against a baffle plate which also serves to remove the yarn from the jet stream.

The action of the jet in untwisting the yarn may be likened to a combing action. The pull of the jet stream acts to straighten the helically twisted fibers, creating a torque which untwists the yarn. A jet operated at near sonic velocity provides sufficient torque to untwist the yarns usually encountered, but it is sometimes desirable, especially with high twist single ply yarn, to provide a rotating torque jet which rotates in the opposite direction from that of the yarn twist to accentuate the false untwisting torque of the jet. Purely mechanical means for applying false twist are known in the art, but are not necessary to accomplish the false untwist described. After the fibers have been untwisted the turbulence of a high velocity jet will act to separate the fibers and form them individually into convolutions with outwardly projecting fiber ends. Both staple yarn and continuous filament yarn can therefore be processed in a similar manner with a near sonic velocity jet to produce the desired bulky yarn having a covering of projecting fiber ends.

Plied yarn can be processed somewhat more readily than single ply yarn because the plies exert a snubbing action on each other which tends to resist untwisting of the fibers. This effect can supply a part or all of the snubbing action required to prevent the region of false untwist from being so extensive that the yarn is pulled apart. This is most easily seen in the case of a plied staple yarn of the usual type in which the singles twist is in one direction, e. g., a **Z** twist, and the ply twist is in the opposite direction, e. g., an **S** twist. An untwisting torque applied to the ply fibers also causes the plies to twist together in the opposite direction, which increase of ply twist opposes the above torque and tends to prevent the fibers from being separated for more than a short distance. If the twist is sufficiently great, as in a high twist yarn, this opposition to fiber separation provides all of the snubbing needed and it is not necessary to rely on snubbing surfaces before and after the jet. The same

thing is true to a lesser extent when the plies fed to the jet are not twisted together. The plies still provide a snubbing action which opposes forces tending to untwist the fibers of a ply. Thus two separate single ply yarns can be fed to a jet together and processed into a single yarn in accordance with this invention with less difficulty than a single ply. When one ply is composed of continuous filaments and another ply is composed of staple-length fibers, the continuous filaments also help resist tensions tending to exceed the draft yield strength 10 of the staple ply.

Figure 1 shows a suitable arrangement of apparatus for practicing the process of this invention. The starting yarn 10 may be supplied from any convenient source, such as a yarn package, and may come directly from the spinning process by which it is produced without intermediate wind-up. The yarn is passed between feed rolls 12 and 14, arranged to be driven so as to forward the yarn at the desired speed, which is preferably of the order of 50 to 100 yards per minute but may vary over a wide range. These feed rolls are mounted on a pedestal 16. The yarn passes through guide 18 on support 20 and into a jet nozzle supported by air supply pipe 22. The nozzle is shown in section to clarify the construction. The body portion 24 of the nozzle is hollow and is provided with a fluid exit 26 which has a venturi-like shape to create the required high velocity jet. A hollow male member 28 is threaded into the body at 30 and terminates in a cone 32 projecting into the mouth of the jet-forming exit 26. The yarn passes inside the male member, out through a hole in the projecting cone, and is carried out of the nozzle exit 26 by the jet stream created by air entering the nozzle through pipe 22. The flow of air to the jet can be regulated by valve 34 in the supply pipe. The yarn hole in cone 32 should be of a size which provides a fairly snug fit around the yarn so that the yarn is snubbed sufficiently to prevent appreciable untwisting before the jet is reached, unless equivalent snubbing is provided by other means.

The yarn leaving the nozzle is deflected at right angles by a baffle plate 36 mounted on the nozzle close to the exit 26. The baffle plate accomplishes the dual purpose of terminating the action of the high velocity jet on the yarn and of snubbing the yarn against untwisting beyond this point. For reasons previously explained, the distance from the end of the cone 32 to the baffle plate must be less than the length of fibers in the treated yarn, and should preferably be such as to limit the false untwisting action of the jet to less than one-half the fiber length. Instead of the baffle plate, a guide can be used to achieve a similar result. Frequently sufficient snubbing can be accomplished by pulling the yarn across exit face 38 of the nozzle. When sufficient back snubbing is not provided by the yarn hole in cone 32 the yarn can be fed into the nozzle at an angle so that the yarn is snubbed against other parts of the male member 28.

The jet stream is operated at a near sonic velocity to separate the fibers, form them into bulk-giving convolutions, and cause fiber ends to project from the yarn, all as described previously. The treated yarn now passes through a guide 40 located below baffle 36, and then to a pair of take-up rolls 44 and 46, which are suitably supported on pedestal 42 and are driven at a surface speed somewhat less than that of feed rolls 12, 14 to provide an overfeed to the jet. The amount of overfeed is one of the factors controlling the amount of bulking action accomplished in the jet and should generally be in the range of 5% to 50%, depending upon the effect desired. The percent overfeed is the percent by which the speed of yarn feed to the jet exceeds the take-up speed. The take-up rolls 44, 46 may feed to any suitable wind-up or, alternatively, one of these rolls can be a wind-up roll.

A variety of nozzles can be used instead of the one illustrated in Figure 1 to provide the required jet. A simple alternative form is shown in Figures 2 and 3. A metal block 50 is drilled lengthwise to provide axial yarn passage 52. An air entrance 54 is drilled at a forward

angle of about 45° through one face of the block to intercept the yarn passage. When a rotating jet stream is desired the air entrance may be made of smaller diameter than the yarn passage and be off center to intercept the 5 yarn passage at one side as shown in Figure 3. Fitting 56 is soldered over the air entrance; it is threaded at 58 for attachment to the air supply pipe 22 of the apparatus shown in Figure 1. In place of air other fluids can be used such as CO<sub>2</sub>, steam, or other vapors for special purposes.

The nozzle shown in Figure 4 provides advantages over the two forms already described. The housing 60 may be a standard 1/4 inch plumber's T. The yarn enters through guide member 61, provided with a funnel-shaped portion 62 to receive the yarn end when stringing up. A hypodermic needle 63 of appropriate size provides a passage for conducting the yarn into the nozzle 64. The nozzle has the shape of a conventional venturi tube with the entrance 65 tapering inward so that opposite sides are at about a 20° angle with each other, and the exit 66 diverging more gradually so that opposite sides are at about a 7° angle with each other. The overall length of the venturi tube may suitably be about 1.3 inches with the diverging exit portion about 1.0 inch long. The arrangement of guide member 61, needle passage 63 and nozzle 64 makes the device self-stringing when a yarn end is fed to it.

The needle 63 is adjusted to extend into the entrance of the venturi and stop in the venturi throat 67. This adjustment is important for best performance. The manner of adjustment shown is to thread the outside of the nozzle and provide positioning and locking nuts 68, 69. The nozzle slides with a snug fit into the housing 60 until nut 68 rests against the housing. It is held in this position by 30 springs, one of which is indicated at 73. The guide member 61 likewise slides into the housing with a snug fit until shoulder 71 is positioned against the housing. It may also be held in position by spring 70 and other similar springs. Advantages of this construction are that it can be taken 35 apart easily for cleaning and the parts can be rotated to adjust the needle in the venturi throat. However, either or both parts may be held in position by set screws passing through the housing, or the parts may be threaded into the housing.

Air is supplied to the nozzle through pipe 72, which is threaded or soldered into the T housing. The air passes through the venturi around the needle 63, the venturi throat 67 being sufficiently larger than the needle to permit passage of the required volume of air. Gasket material may be placed in groove 73 around member 61 and groove 74 around the nozzle to prevent air leakage.

In Figure 13, 1 represents a flock chamber provided with an inlet 2 and an exit 3 for the yarn. Between the inlet and exit is an open space containing flock 7. The chamber is also provided with an internal air baffle. The air supplied through the texturing jet keeps the flock or linters in a state of violent agitation. The inlet 2 is usually through a texturing jet which is provided with an air supply 4 and an outlet 5 at the base of a venturi chamber 6.

The yarn is led through the inlet 2 where it is subjected to a high speed air jet which textures the yarn forming whorls and loops. As the yarn passes through the suspended flock 7, the fibers find their way into the interstices and loops of the yarn where they are held and entrained as the yarn passes through the exit 3 of the flocking chamber 1. The yarn then proceeds as shown in Figure 14.

The process and products of the invention will now be illustrated by the following examples, which are not to be construed as limiting the scope of the invention.

#### EXAMPLE 1

The apparatus shown in Figure 1 was used to process a single ply of 150 denier, 40 filament, 0 twist, continuous filament cellulose acetate yarn. This yarn was fed to the nozzle at 60 yards per minute and taken up after treatment

ment at 40 yards per minute, an overfeed of 50%. Air was supplied to the nozzle at 90 pounds per square inch gage pressure to give an effective jet velocity of slightly greater than sonic, and an air flow through the nozzle of 2.6 cubic feet per minute measured as "free" air at atmospheric pressure and temperature. The baffle plate was spaced  $\frac{1}{8}$  inch from the nozzle exit. The appearance of the untwisted treated yarn is shown in Figure 5. The filaments were convoluted and partially shattered to provide a multitude of filament loops and protruding ends as shown. This yarn was rather weak.

Two plies of the above yarn were fed together to the nozzle at 19 yards per minute and taken up after treatment at 14 yards per minute, an overfeed of 36%. The other conditions were the same as above. Figure 6 shows the appearance of this two-ply yarn after treatment, which exhibited the characteristic fiber loops and ends described above. When twisted the yarn was reasonably strong and processed satisfactorily into fabric.

Operation of the process as above, but without the baffle plate, or with the baffle plate spaced one inch or more from the nozzle exit, resulted in the yarn being completely shattered into flock. Operation of the process as above, but at air pressures of 40 pounds per square inch to give air flows of less than 1.0 cubic feet per minute, measured as free air, produced bulk-giving convolutions without appreciable filament shattering, whereas pressures of 50 or more pounds per square inch produced the multitude of filament loops and ends described above.

#### EXAMPLE 2

Using the apparatus shown in Figure 1, two separate plies of yarn were fed to the nozzle. One ply was a 20 cotton count, 15 Z twist (15 turns per inch) cotton yarn. The other ply was a 200 denier, 80 filament, continuous filament acrylonitrile yarn. The yarns were fed into the nozzle together at 10 yards per minute. Air was supplied to the nozzle at 90 pounds per square inch gage pressure, which gave a flow, as free air, of 2.7 cubic feet per minute. The appearance of the resulting two-ply yarn after receiving a slight twist is shown in Figure 7. The bulk of both plies was markedly increased by the formation of crunodal loops and other convolutions, and cotton fibers were caused to project with a great increase in fuzziness. The cotton ply was extended in length by the treatment, so that it wrapped around the continuous filament ply when the yarn was twisted.

An attempt to treat the cotton yarn alone under similar conditions, but without the baffle plate, resulted in the yarn being completely blown apart and reverted to unspun staple. The same was true even under such relatively mild conditions as 50 pounds per square inch air pressure and 10% overfeed; the cotton yarn was disintegrated.

#### EXAMPLE 3

A single ply, 18 cotton count, 18 Z twist spun yarn composed of 3-inch staple length, 3 denier, acrylonitrile fibers was processed with an apparatus similar to that shown in Figure 1. The yarn was taken up from the nozzle at 15 yards per minute and the baffle plate was located  $\frac{3}{4}$  inch from the snub point provided by the restricted yarn passage into the jet stream. Air was supplied to the nozzle at 90 pounds per square inch gage, the nozzle dimensions being such as to give a flow of about 1 cubic foot per minute with an effective jet stream velocity of slightly above sonic velocity. The appearance of the treated yarn is shown in Figure 8. The yarn was greatly increased in bulk and the surface was covered with ring-like loops and extending fiber ends, giving the yarn a fuzzy or lofty appearance and feel.

#### EXAMPLE 4

A single ply, 18 cotton count, 14 Z twist spun yarn composed of  $4\frac{1}{2}$  inch staple length, 3 denier, acrylonitrile fibers was processed at about 100 yards per min-

ute and 10% overfeed using an air pressure of 50 pounds per square inch gage. The apparatus was similar to that shown in Figure 1, except that the nozzle shown in Figure 4 was used without a baffle plate and yarn guide 40 was located beside the nozzle so that the yarn was snubbed across the exit face of the nozzle. The appearance of the treated yarn was as in Figure 8. The denier of the yarn was increased from 323 to 356. The effective volume of the yarn was increased to a much greater extent, resulting in a lofty, fuzzy yarn which has aesthetic merit, particularly for knitted fabrics. The changes in the yarn structure comprise a separation and reorientation of the fibers in relation to each other accompanied by intertwining to the extent that the reoriented fibers are stabilized in their new positions. The net result is a peripheral expansion of the central core of the yarn with an accompanying marked increase in the number and length of free fiber ends and the formation of crunodal loops and other convolutions characteristic of the process. Some properties of fabrics prepared from the untreated and the treated yarn were as follows:

#### Fabric properties

|                           | Before Bulking | After Bulking |
|---------------------------|----------------|---------------|
| Weight (oz./sq. yd.)      | 7.1            | 7.2           |
| Thickness (cm.)           | 0.155          | 0.208         |
| Specific volume (cc./gm.) | 6.45           | 8.55          |

#### EXAMPLE 5

A variety of spun yarns were treated in a similar way with like results. The treated yarns were all taken up from the jet at 100 yards per minute, with other conditions as in Example 4 except as indicated in Table 1. In this table, yarn notations such as 50/2 (25 Z, 4 S ply) 5 in., 3 d. p. f. in 5(e) refer to a 50 cotton count, 2 ply yarn in which each of the plies has a Z twist of 25 turns per inch and the plies are twisted together in the opposite direction at 4 S turns per inch, the fibers being 5 inches long and of 3 denier per fiber. "Rayon" refers to regenerated cellulose yarn made by the viscose process. "Dacron" and "Orlon" are trademarks for yarn manufactured by E. I. du Pont de Nemours and Company and refer to polyethylene-terephthalate and polyacrylonitrile yarns, respectively. "Nylon" refers to polyhexamethyleneadipamide yarn. The appearance of the treated yarns was similar to that shown in Figure 8. However, it was observed that, as the staple length was increased, the amount of loop formation in the yarn bundle increased and, of course, the frequency of protruding ends decreased. The extent of the bulking action could be increased or decreased by varying the per cent overfeed up or down from the values given in the table, but processing difficulties may be encountered at overfeeds above 15%.

TABLE I.—PREFERRED PROCESS CONDITIONS FOR BULKING SPUN YARNS

| Ex.   | Yarn Treated                                                          | Overfeed, Percent | Air Pressure, lbs./sq. in. |
|-------|-----------------------------------------------------------------------|-------------------|----------------------------|
| 5 (a) | 18/1(14 Z) 8-10 in., 3 d. p. f. Rayon                                 | 18                | 50-70                      |
| 5 (b) | 30/1(19 Z) 3.5 in., 3 d. p. f. Rayon                                  | 5                 | 40-60                      |
| 5 (c) | 40/1(22 Z) 6-8 in., 3 d. p. f. Rayon                                  | 10                | 60-80                      |
| 5 (d) | 10/1(11 Z) 5 in., 3 d. p. f. "Dacron"                                 | 6                 | 60-80                      |
| 5 (e) | 50/2 (25 Z, 4 S ply) 5 in., 3 d. p. f.                                | 6                 | 60-80                      |
| 5 (f) | 18/1(15 Z) 4-6 in., 2.5 d. p. f. Nylon                                | 6                 | 60-80                      |
| 5 (g) | 15/1(14 Z) 4 in., 3 d. p. f. blend of 50% "Dacron", 50% Rayon fibers. | 5                 | 50-70                      |

#### EXAMPLE 6

A 20/1 worsted count (408 total denier) 9 Z twist spun yarn composed of 5 inch, 3 denier, acrylonitrile fibers was processed with the apparatus shown in Fig-

ure 1 at a speed of 15.5 yards per minute. Air was supplied to the nozzle at a pressure of 90 pounds per square inch gage, the air consumption being 2.44 cubic feet of free air per minute. The treated yarn was characterized by the protrusion of long ends of fibers from the core of the yarn. These ends projected up to one inch, giving an extremely fuzzy, cashmere-like yarn. In other respects the yarn was similar to that shown in Figure 8.

## EXAMPLE 7

A two ply, 27 cotton count, spun polyethylene-terephthalate yarn was processed at 15 yards per minute with apparatus similar to that in Figure 1. The plies of this yarn were composed of  $1\frac{3}{4}$  inch staple length, 3 denier fibers twisted together at 18 Z turns per inch, and the ply twist was 11 S. Air was supplied to the nozzle at 90 pounds per square inch gage, the flow being about 1 cubic foot of free air per minute. The yarn bulked equally well both with and without the baffle plate. The appearance of the yarn is shown in Figure 9 and, except for the two-ply structure, was similar to the yarns described previously in connection with Figure 8. In this case the fiber and ply twists were sufficient to prevent the false untwist imparted by the jet from untwisting the yarn fibers for an undesirable distance, and snubbing against a surface was not necessary.

An attempt was made to process a single ply, 27 cotton count, 18 Z twist yarn composed of  $1\frac{3}{4}$  inch, 3 denier polyethyleneterephthalate fibers under identical conditions. Without the baffle plate, or other means for snubbing the yarn close to the nozzle exit, the process could not be operated because the air stream pulled the yarn to pieces.

## EXAMPLE 8

The previous examples have shown that the jet stream has sufficient false untwisting action to open up a wide variety of twisted yarns to the extent required by the process of this invention. However, it is sometimes desirable to accentuate the untwisting action by providing a rotating or torque jet stream. This has been accomplished by cutting oblique or spiralling grooves in the cone-shaped end 32 of the yarn guiding portion of the nozzle in Figure 1. For the purposes of the present example, however, the simple torque nozzle shown in Figures 2 and 3 was used with apparatus similar to that of Figure 1 to process single ply, 18 cotton count, 18 Z twist, spun yarn composed of 3 inch, 3 denier polyacrylonitrile fibers. Air was supplied at 90 pounds per square inch gage to give a flow at near sonic velocity of  $\frac{1}{2}$  cubic foot of free air per minute.

Using a nozzle having a  $\frac{1}{16}$ -inch yarn passage and arranged to apply an S torque to yarn being treated, with the yarn snubbed  $\frac{1}{4}$  inch from the nozzle exit at a distance of 1 inch from the air inlet and then taken up at 15 yards per minute, the Z twist yarn processed excellently to give a multitude of ring-like loops and fuzzy ends. The yarn processed better than the same yarn did in the straight-line jet stream of Example 3, even though the air consumption was only one-half as great. This nozzle appeared as in Figure 3 when looking upstream at the nozzle exit. The air inlet 54 was off center to the left, giving the air stream a clockwise rotation as it came toward the observer.

An attempt was made to use a nozzle with the air inlet off center to the right, which gave a counterclockwise rotation to the air stream and applied a Z torque to the yarn, but this had no appreciable effect on the yarn. This Z torque jet increased the Z twist of the yarn and prevented the opening action necessary for the type of 70 bulking action described.

Cotton yarn also processed excellently under the above conditions with the S torque jet. Good results were obtained with a single ply, 18 Z twist cotton yarn having an average fiber length of  $1\frac{5}{16}$  inches. Due to the short

fiber length the bulking effect was somewhat less than for the above 3-inch fiber length polyacrylonitrile yarn. When an attempt was made to treat the cotton yarn with the snubbing point over 1 inch from the nozzle, under otherwise identical conditions, the process was not operable because the yarn pulled apart.

## EXAMPLE 9

In Example 8 it was observed that the use of a Z torque jet nozzle increased the twist of the Z twist yarn and prevented opening of the yarn, so that bulking did not take place. However, this type of treatment can be combined with heat-setting of the yarn while in the over-twisted condition to provide a crimp bulking effect. A single ply, 18 cotton count, 15 Z twist spun yarn composed of 4-6 inch, 2.5 denier, polyhexamethylene adipamide fibers may be processed as in Example 8, using a torque nozzle which applies a false twist of about 30 turns per inch. The nozzle may be heated to about 240-250° C. to crimp set the yarn while in the false twisted condition. This produces a bulky wool-like yarn having an attractive curly crimp which imparts elasticity to the yarn. The fibers will retain their crimp when separated from the yarn.

It will often be more convenient to heat the false twisted yarn outside of the nozzle instead of heating the torque nozzle. The yarn guide 18 was spaced at a greater distance from the nozzle than shown in Figure 1 and a heating surface at 240-250° C. was used to crimp set the yarn between the guide and the nozzle. The yarn was passed through the torque nozzle without snubbing so that the false twist of about 30 turns per inch backed up to the yarn guide. With other conditions as described above, a similar crimp bulking effect was obtained.

The process of Example 9 is useful with any yarn composed of fibers which can be heat set to stabilize the crimp imparted by the false twist. The treatment is enhanced by fibers which shrink during heat-setting. While the process has been illustrated with spun staple yarn, it is equally applicable to continuous filament yarns, both twisted and untwisted. The process can be combined with the treatments of any of the other examples by adding another nozzle to apply a separate false untwisting and bulking step.

## EXAMPLE 10

A nylon yarn (80/68/0) was fed to a jet similar to Figure 8 of U. S. 2,783,609 at 240 Y. P. M. The jet was mounted so as to exhaust in an enclosure partly filled with cotton linters of about  $\frac{1}{16}$  in length (Figures 13 and 14). The pinch rolls as illustrated in Figure 14 were operated at 200 Y. P. M. to give an intermediate overfeed of 20%. The wind-up was operated at 230 Y. P. M. to give a net overfeed of 5% and a final denier of 91. Since the calculated denier under these conditions should be 84, the linters increased the yarn weight by about 8%. The yarn sample between the flocking box and the pinch rolls had an appearance illustrated in Figure 15. The final yarn showed reduced loop size as shown in Figure 16. Many characteristic random nodes and tangles could be observed under magnification. The short length staple fibers were firmly locked within a continuous filament knot or knot snarl or tangle of random configuration and frequently compound in structure; that is, more than one continuous filament and more than one staple fiber involved in a given snarl or tangle. Longer fibers may be used in place of those used to illustrate the invention in this example. In general the flock or linters may vary in length from about 0.1 millimeter, as is usually found in wood flour, up to lengths normally employed for staple fibers; that is, about 15 millimeters, although for many purposes staple up to about 5" may be used. In general the shorter length fibers are loosely bound and have a tendency to be lost in yarn and fabric processing. Fibers of normal staple length in the range

of 1" to 3" are entangled less readily by the bulked yarn and therefore tend to modify the yarn to a lesser extent in terms of the number of free ends. Longer fibers, however, have the advantage of being more permanent in the final fabric.

Any process which tends to entangle the longer fibers in the bulked continuous filament yarn may be used to advantage where the staple is long, for example, it may be desirable to pass the bulked yarn through a loosely compacted bat of randomly arranged fibers. The length of contact and compressional load on the yarn being treated should be balanced to avoid undue yarn tension tending to cause breakdowns but may be sufficient to cause filament loops to become locked about the entangled staple fibers and to deform large loops into the flattened configuration shown in Figure 17. Protruding fibers and elongated loops may be held temporarily in place by a size to improve weaving performance and reduce snagging characteristics in the final fabric.

Where improved yarn stability is the major goal, short length fibers such as Solka-Floc<sup>1</sup> wood cellulose may be employed with good results. The very short length fibers tend to be fugitive to some extent but increase stability of borderline yarns sufficiently to permit improved warping, quilling and weaving or knitting. The bulk of the finished fabrics may be enhanced even after loss of the short fibers due to the unoccupied spaces they leave behind.

Similarly, the bulked yarn may be passed through a liquid fiber slurry. With well dispersed fibrous material of suitable length and concentration the yarn emerges with much the appearance of a pipe cleaner and increased weight of up to 50% or more. Tension applied to this yarn may again be used to lock most of these fibers in place. Heavily loaded yarns tend, however, to lose a portion of the loosely attached fibers which may be blown, rubbed or shaken off and returned to the slurry.

The following experiments illustrate embodiments of the invention in which two different yarns are used, one of which is relatively shatterable and the other is relatively unshatterable.

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100<br

In general, with other factors held constant, the tougher fibers may be stabilized by use of lower operating speed on the jet so that the individual increments of fiber length are exposed to the flexing action of the jet for a greater length of time, or by use of higher air pressure in the jet which gives a more violent flexing action in the jet. An example of the former deals with rayon which was processed at 20 Y. P. M. to give a product similar to that obtained with acetate at 200 Y. P. M. (roughly in inverse proportion to the tabulated flex lives).

Within a given fiber composition, a great range of flex lives may be obtained by changes in orientation and/or crystallinity. Normally, nylon and "Dacron" are much too tough to be fractured by the action of a texturing jet. If, however, they are prepared in a state of low orientation and high crystallinity the flex lives may be reduced to the range of a few hundred to a few thousand cycles. Molecular weight as indicated by relative viscosity in a suitable solvent also plays an important part in determining fiber toughness. "Dacron" fibers prepared from polymer with a relative viscosity of about 12 even though oriented and crystallized by normal process steps show flex lives in this same low range (100-10,000). Usually a filament having a flex life below about 10,000 may be substituted for the acetate in the examples.

Some of the examples and the disclosure illustrate the use of a torque nozzle to process the product of this invention. It is to be understood that this treatment and the torque nozzle per se do not form a part of the present invention since they are disclosed and claimed in copending applications.

Since many different embodiments of the invention may be made without departing from the spirit and scope thereof, it is to be understood that the invention is not limited by the specific illustrations except to the extent defined in the following claims.

I claim:

1. A bulky yarn comprising a plurality of discontinuous fibers twisted together, the fibers being convoluted into coils, loops and whorls at random intervals along their lengths, and the yarn surface exhibiting a multitude of ring-like loops and protruding fiber ends irregularly spaced along the yarn surface.

2. A bulky yarn comprising a plurality of twisted staple-length fibers which are individually looped upon themselves at random intervals along their lengths and at ir-

regular spacing on different fibers, said yarn exhibiting a fuzzy surface composed of protruding fiber ends and crunodal loops.

3. A bulky twisted staple yarn characterized by having a multitude of ring-like loops and protruding fiber ends irregularly spaced along the yarn surface and having a multitude of fiber convolutions irregularly scattered through the yarn structure providing a bulk-giving lateral interfiber spacing.

4. A bulky yarn composed of at least two plies of twisted staple fiber characterized by having a multitude of ring-like loops and protruding fiber ends irregularly spaced along the yarn surface and having a multitude of fiber convolutions irregularly scattered through the yarn structure providing a bulk-giving lateral interfiber spacing.

5. A bulky yarn having a fuzzy surface formed by a multitude of protruding fiber ends and having a multitude of crunodal loops and other convolutions irregularly scattered through the yarn structure providing a bulk-giving lateral interfiber spacing.

6. A bulky yarn having a fuzzy surface formed by protruding ends of staple fiber and having a core structure comprising substantially continuous filaments which are individually convoluted into coils, loops and whorls at random intervals along their lengths and characterized by the presence of a multitude of crunodal loops.

7. A bulky yarn having a large number of protruding free ends of fiber and an enhanced bulk provided by crunodal loops and other fiber convolutions scattered through the yarn structure, the yarn fibers being twisted together to hold the structure in place.

8. A bulky twisted yarn having a multitude of fiber ends protruding from the surface and comprising a plurality of staple-length fibers which are individually looped upon themselves at random intervals along their lengths and irregularly spaced on different fibers, which loops substantially disappear when the yarn is untwisted and pulled apart.

#### References Cited in the file of this patent

#### UNITED STATES PATENTS

|           |                   |       |               |
|-----------|-------------------|-------|---------------|
| 2,199,400 | Geier et al.      | ----- | May 7, 1940   |
| 2,293,003 | Hunter            | ----- | Aug. 11, 1942 |
| 2,344,892 | Modigliani et al. | ----- | Mar. 21, 1944 |
| 2,581,566 | Whitehead et al.  | ----- | Jan. 8, 1952  |